

# United States Patent

[19]

Tanaka et al.

[11] 3,889,033

[45] June 10, 1975

[54] **TRANSFERRING PAPER FOR ELECTROPHOTOGRAPHY**

[75] Inventors: **Hiroshi Tanaka; Ikuo Soma**, both of Tokyo; **Yoshikazu Ito; Masayasu Kamijo**, both of Fuji, all of Japan

[73] Assignee: **Canon Kabushiki Kaisha**, Tokyo, Japan

[22] Filed: **Mar. 1, 1973**

[21] Appl. No.: **337,118**

[30] **Foreign Application Priority Data**

Mar. 3, 1972 Japan ..... 47-22002

[52] U.S. Cl. ..... **428/323**; 96/1 R; 96/1 LY;  
96/1.4; 428/331

[51] Int. Cl. ..... **D21h 1/28**

[58] **Field of Search** ..... 96/1 R, 1 LY, 1.4;  
117/155 UA, 161 UC, 161 UD, 161 UB, 161  
UH, 37 LE

[56] **References Cited**

UNITED STATES PATENTS

3,234,017 2/1966 Heyl et al. ..... 96/1 R

|           |         |                      |        |
|-----------|---------|----------------------|--------|
| 3,414,410 | 12/1968 | Bartlett et al. .... | 96/1 X |
| 3,554,747 | 1/1971  | Dastoor .....        | 96/1 X |
| 3,582,321 | 6/1971  | Ueda et al. ....     | 96/1 X |
| 3,642,480 | 2/1972  | Urancken .....       | 96/1 X |
| 3,681,069 | 8/1972  | McNamee et al. ....  | 96/1 X |

*Primary Examiner*—Michael R. Lusignan  
*Attorney, Agent, or Firm*—Fitzpatrick, Cella, Harper  
& Scinto

[57]

## ABSTRACT

A transferring paper for an electrophotographic process comprising developing an electric latent image with a liquid developer and transferring the image thus developed comprises a base paper and a coating layer produced by coating on the base paper a coating agent composed of 50 – 500 parts (as solid) of polymer emulsion having a second order transition temperature of from –40°C to 25°C as a binder and 100 parts of a white inorganic filler at an amount of 2 – 10 g./m<sup>2</sup>. (as solid), carrier resistance of the resulting transferring surface being 1.5 – 15 sec., smoothness of the resulting transferring surface being 30 – 300 sec. and density being 0.75 – 1.00 g./cm<sup>3</sup>.

5 Claims, 4 Drawing Figures



FIG. 1



FIG. 2



FIG. 3



FIG. 4



TRANSFERRING PAPER FOR  
ELECTROPHOTOGRAPHY

## BACKGROUND OF THE INVENTION

## 1. Field of the Invention

This invention relates to a transferring paper for electrophotography used for transferring a developed image obtained by developing an electric latent image produced on an electrophotographic photosensitive member or insulating layer with a liquid developer.

## 2. Description of the Prior Art

Heretofore, there are known methods of transferring to a transferring paper an image obtained by developing an electric latent image formed on an electrophotographic photosensitive member with a liquid developer. For example, Japanese Patent Publication No. 24077/1970 discloses an electrophotographic method which comprises applying a blanket corona charging to a photosensitive plate composed of a support such as aluminum plate, a photoconductive layer (CdS-binder system etc.) overlying the support and an insulating layer overlying the photoconductive layer, imagewise exposing simultaneously with applying a corona charging of a polarity opposite to that of the blanket corona charging or AC corona charging, applying a blanket irradiation to produce an electric latent image, developing the resulting electric latent image with a liquid developer, and transferring the resulting developed image to a transferring paper.

A transferring paper for transferring a toner image obtained by developing an electric latent image with a dry developing agent has been already known and disclosed in Japanese Patent Publication No. 20152/1966 and others, but such transferring paper can not be used for transferring of an image developed with a liquid developer. A new transferring paper for liquid development has been demanded.

## SUMMARY OF THE INVENTION

According to the present invention there is provided a transferring paper to which an image obtained by developing an electric latent image on an electrophotographic photosensitive member with a liquid developer is transferred, which comprises a base paper and a coating layer thereon in an amount of 2 - 10 g./m<sup>2</sup>, composed of 50 - 500 parts by weight of a polymer having a second order transition temperature of -40°C to 25°C and 100 parts by weight of a white inorganic filler, the carrier resistance of the transferring surface being 1.5 to 15 sec., the smoothness of the transferring surface being 30 to 300 sec. according to the measuring method as defined in the specification, and the density being 0.95 to 1.00 g./cm<sup>3</sup>.

An object of this invention is to provide a transferring paper of good transferability to which an image obtained by developing an electric latent image on an electrophotographic photosensitive member with a liquid developer is transferred.

Another object of this invention is to provide the transferring paper of excellent fixation of a transferred image.

A further object of this invention is to provide the transferring paper consuming less amount of a liquid developer and of good drying property.

## BRIEF DESCRIPTION OF THE DRAWINGS

FIG. 1 shows an apparatus of measuring a carrier resistance;

5 FIG. 2 is a graph showing a relation between a carrier resistance and a second order transition temperature (Tg value);

FIG. 3 is a graph showing a relation between density of a transferred image and a carrier resistance; and

10 FIG. 4 is a graph showing a relation between density of a transferred image and smoothness of the surface.

DESCRIPTION OF THE PREFERRED  
EMBODIMENT

15 The present inventors have now found that a transferring paper for images obtained by liquid developing should have the following various properties.

## 1. Carrier Resistance

As a carrier for a liquid developer, there may be used 20 a carrier used in conventional wet developing process for electrophotography and electrostatic recording. The liquid is a highly electric resistant organic solvent of volume resistivity of higher than 10<sup>10</sup> Ohm-cm and dielectric constant of less than 3, which does not destroy an electrostatic image, such as paraffin organic solvents, for example, liquid paraffin and liquid isoparaffin. As commercially available isoparaffin organic solvents, there may be mentioned Isopar H, G and L supplied by ESSO.

30 What is meant by "carrier resistance" in the present invention is a resistance to penetration of a paraffin organic solvent such as, for example, Isopar as used for liquid developer.

When a transferring paper does not have a carrier resistance or have only insufficient carrier resistance, a carrier liquid penetrates a transferring paper upon transferring so that a sufficient electrophoresis transferring can not be effected and the resulting transferred image is blurred. Furthermore, much liquid developer 40 is consumed and drying property is lowered so that there is a problem in practical operation.

During transferring, it is desirable to soften a material capable of imparting carrier resistance at the interface between the developer and the liquid carrier and accept a coloring matter such as pigment material from the developer.

When the carrier resistance is too strong, the affinity to a carrier liquid is so lowered that fixation of the transferred image is not good and the transferred image 50 is often smudged by friction even after drying.

As is clear from above, it is necessary that the transferring paper has an appropriate degree of carrier resistance. Degree of carrier resistance is determined by the following method according to the present invention, and an appropriate carrier resistance range is defined by the value determined by the method.

Referring to FIG. 1, a sample for measuring 1 is set to a metal frame 2, and an injector 4 for dropping a carrier liquid is horizontally fixed to a support 6. A micrometer 5 is gradually rotated to drop 1 drop of a carrier liquid ("Isopar G," supplied by ESSO) to a circle of 7 mm in dia. on the sample paper. When the carrier liquid arrives at the sample, a stopwatch is actuated and then stopped when the one drop of carrier liquid penetrates over the whole area of the circle 3 of 7 mm. in dia. and the portion of the paper has become transparent. The period of time thus measured is used as a de-

gree of carrier resistance. The distance between the injector needle and the sample surface is about 2 cm. When a carrier liquid is dropped to a paper having no carrier resistance according to the above mentioned method, the carrier liquid instantly penetrates and spreads to the full size of area for 1 drop. On the contrary, when a sample paper having carrier resistance is used, it takes some time depending upon the degree of carrier resistance that the carrier liquid penetrates and spread to the full size of area for one drop. The injector for dropping a carrier liquid is that of 1 cc. or 2 cc. and the needle is a type of 1/3. The volume of one drop under the above mentioned condition is about 0.004 cc.

The practical degree of carrier resistance as measured by the above mentioned method is from 1.5 to 15 sec., preferred with from about 2 to 10 sec. This will be explained in connection with Examples.

### 2. Smoothness

Smoothness of transferring papers having an appropriate degree of carrier resistance has been measured by Bekk tester for paper according to JIS P8119 and it has now been found that smoothness ranging from 30 sec. to 300 sec., preferred with 40 sec. to 200 sec. is appropriate.

When smoothness of the paper is lower than 30 sec., there occurs irregular transferring to fail to produce a good transferred image unless a large amount of a liquid developer is present, and it takes a long time to dry the liquid developer.

When smoothness is higher than 300 sec., a good transferred image can be obtained by only a small amount of liquid developer, but fixation of the developer after transferred is not good and the image is disadvantageously damaged by friction. This will be further explained by referring to experimental data.

### 3. Density

Most important properties of transferring paper are carrier resistance and smoothness. In addition, density of a transferring paper is also important which is related to carrier resistance and smoothness.

Density of paper varies depending upon degree of beating, composition of coating agent, amount of coating agent, conditions of calender or supercalender. In order to improve carrier resistance of a transferring paper, a porous paper is not preferable. As the result of research, it has now been found that density of the transferring paper should be higher than 0.75 g./cm<sup>3</sup>, preferred with higher than 0.78 g./cm<sup>3</sup>.

On the other hand, it has been now further found that density of transferring paper of good fixation should be less than 1.00 g./cm<sup>3</sup>, preferred with less than 0.97 g./cm<sup>3</sup>, when the smoothness is lower than 300 sec. and the coating agent of the present invention is employed.

In view of the foregoing, preferable density for the transferring paper ranges from 0.75 to 1.00 g./cm<sup>3</sup>.

Density of paper is calculated according to the following formula,

$$\text{density (g./cm}^3\text{)} = \frac{W}{T \times 1000}$$

wherein W is a basic weight (g./m<sup>2</sup>) determined according to JIS P 8124 and T is thickness (mm.). The thickness T is determined by using a micrometer ac-

cording to JIS P 8118, i.e. a diameter of the smaller one of two planes being about 14 mm.

In order to obtain an excellent transferring paper of good fixability satisfying carrier resistance and smoothness according to the above mentioned measuring method, it is necessary to provide a coating layer of good film shaping state after coating and drying.

Since, among various solvents, paraffin series solvents g./m as Isopar usually used for liquid developer can particularly easily penetrate a paper layer, the carrier resistance mainly depends on the film forming state of the surface coating layer, i.e. barrier property, but not on thickness and basic weight of paper as far as the basic weight is in a range of that of usual copying paper. At a basic weight higher than 100 g./m<sup>2</sup>, the thickness of the paper affects the carrier resistance. At a basic weight higher than 150 g./cm<sup>2</sup>, the carrier resistance becomes higher than 2 - 4 sec. by the effect of thickness of paper and basic weight even when the barrier property of the coating layer itself is not sufficient. On the contrary, sometimes a carrier resistance is higher than 15 sec. though there are given good transferring and fixation. However, the paper used in this invention is usually a paper of basic weight lower than 150 g./m<sup>2</sup>, particularly, lower than 100 g./m<sup>2</sup>.

The coating compositions used in this invention is mainly composed of an inorganic filler and a polymer emulsion binder. For obtaining satisfactory carrier resistance and smoothness, a ratio of the inorganic filler to a binder and the second order transition temperature are very important. The "polymer emulsion" as mentioned above is a general term for the thermoplastic resin emulsions, synthetic rubber latex and the like. In conventional coated paper such as printing paper, there are contained 80 - 90% of white inorganic fillers and 20 - 10% of binder (as solid), that is, inorganic fillers are mainly contained. In printing paper, when a binder occupies most portion of the coating surface, the paper has low acceptability to ink. Therefore, the amount of inorganic filler is usually more than the binder for the purpose of improving the printing property.

The transferring paper of the present invention is fundamentally different from conventional coated paper, that is, the amount of polymer emulsion binders (as solid) is more than that of inorganic fillers. For example, 50 - 500 parts, preferably 100 - 400 parts (as solid), of the polymer emulsion binder is used for 100 parts of the inorganic filler (white). When amount of the binder is less than the above mentioned one, the barrier property is low and the carrier resistance is insufficient. On the contrary, when the amount of the polymer emulsion binder is more than 500 parts, the resulting coating causes a blocking tendency to the back side of the winding-up paper or the roll surface after coating, and thereby, surface of the coating layer is deteriorated and it is different to obtain a desirable property. In this case, as white inorganic filler, a filler of small particle size, particularly, that which does not have coarse particle larger than 3 microns as far as possible, is preferable. For example, there may be mentioned clay for coating paper, titanium oxide, and calcium carbonate.

As a polymer emulsion binder used together with the inorganic filler at the above mentioned ratio, it has been found that a polymer material having a second order transition temperature (Tg value) of from 25°C

to  $-40^{\circ}\text{C}$ , preferred with from  $0^{\circ}\text{C}$  to  $-30^{\circ}\text{C}$ , is suitable.

When an emulsion of polymer having  $T_g$  value of lower than  $25^{\circ}\text{C}$ , preferred with lower than  $0^{\circ}\text{C}$ , polymer is apt to flow when dried after coating. Furthermore, an emulsion of a polymer having lower  $T_g$  value easily migrates to the surface of coating and therefore, barrier property and carrier resistance of the resulting paper is improved. When the surface is smoothened by calender, the inorganic filler particles enters the inner portion of the paper layer and the polymer flows by heat and nip pressure to improve barrier property and lessen the penetration of carrier.

However, when  $T_g$  value is too low such as lower than  $-40^{\circ}\text{C}$ , the coating is sticky even after drying at the above mentioned ratio of binder to inorganic filler, and a part of coating is taken up by the roll surface so that the formation of coating is disturbed.

When a polymer emulsion having  $T_g$  value ranging from  $-40^{\circ}\text{C}$  to  $25^{\circ}\text{C}$ , preferred with from  $-30^{\circ}\text{C}$  to  $0^{\circ}\text{C}$ , is used, the fixation property becomes remarkably good. This cause is considered as follows. After transferring a visible image, a temperature of about  $50^{\circ}\text{C}$  is applied to a paper at a fixation step and therefore, the polymer binder having  $T_g$  value of lower than  $25^{\circ}\text{C}$ , particularly  $0^{\circ}\text{C}$ , is softened by heat to improve the fixing property of toner particles.

An example of relation among  $T_g$  value, fixation and carrier resistance is shown in Table 1 below and FIG. 2.

Table 1

| Tg value                            | Fixing property     |
|-------------------------------------|---------------------|
| $80^{\circ} - 50^{\circ}\text{C}$   | X                   |
| $50^{\circ} - 25^{\circ}\text{C}$   | Δ                   |
| $25^{\circ} - 0^{\circ}\text{C}$    | ○                   |
| $0^{\circ} - -30^{\circ}\text{C}$   | ◎                   |
| $-30^{\circ} - -40^{\circ}\text{C}$ | ○ (somewhat sticky) |
| $-40^{\circ} - -60^{\circ}\text{C}$ | - (very sticky)     |

A small amount of a water soluble polymer may be incorporated to the above mentioned composition comprising a polymer emulsion binder and white filler so long as thermal softening of the polymer binder in the coating is not disturbed. Amount of the water soluble polymer should be adjusted in accordance with  $T_g$  value of emulsion binder and the ratio to inorganic filler. The transferring surface of the transferred paper is coated with the above mentioned coating layer, but the non-transferring portion may be optionally coated with a coating other than the above mentioned one.

However, when both sides of a transferring paper are used for receiving transferred images, the both sides are also coated with the coating according to the present invention. In this case, it is preferable to use a paper containing titanium oxide since an image on the other side is not seen through.

The relations among carrier resistance as defined by the above mentioned measurement, surface smoothness and density of transferred image are shown in FIG. 3 and FIG. 4. The black circle line in the figures corresponds to a case of weak squeezing of a liquid developer (i.e. much liquid developer) while the white circle corresponds to a case of strong squeezing of a liquid developer (i.e. little liquid developer). In practical use, it is preferable to use in a state of little liquid developer (i.e. strong squeezing) since consumption of the liquid

developer is kept low and drying is easy. Therefore, transferring property of a transferring paper is to be judged at the above mentioned strong squeezing state, and the higher the density of transferred image, the better the transferring property.

In FIG. 3, it is clear that the transferring property becomes good as the carrier resistance increases in both cases of white circle and black circle. In case of white circle, the difference of transferring property per difference of carrier resistance is larger than that in case of black circle. Therefore, the carrier resistance as defined above is an important factor for transferring property (particularly, in case of strong squeezing of liquid developer). This support the appropriateness of the above mentioned "at an instant of transferring, it is necessary that the surface of the transferring paper has a barrier property and the transferring is effected accurately and uniformly."

The relation among carrier resistance, smoothness and practicability of transferring paper is shown in Table 2.

Table 2

| Smoothness<br>(sec.) | Carrier resistance (sec.) |       |      |       |                   |
|----------------------|---------------------------|-------|------|-------|-------------------|
|                      | 0-1.5                     | 1.5-4 | 4-10 | 10-15 | higher<br>than 15 |
| lower than<br>30     | X                         | Δ     | Δ    | Δ     | Δ                 |
| 30 - 50              | X                         | ○     | ○    | ○     | Δ                 |
| 50 - 200             | X                         | ○     | ○    | ○     | Δ                 |
| 200 - 300            | X                         | ○     | ○    | ○     | Δ                 |
| higher than<br>300   | X                         | Δ     | Δ    | Δ     | X                 |

◎ Very good

○ Good

Δ Somewhat bad

X Not usable

The following examples are given for illustrating the present invention.

#### EXAMPLE 1

A mixture of nonionic polyvinyl acetate emulsion and clay (solid ratio, 1:2) was coated on a base paper ( $60 \text{ g./m}^2$ ) at an amount of  $7 - 8 \text{ g./m}^2$ . (both side, as solid) by on-machine size press and dried, followed by machine calender treatment. The  $T_g$  value of emulsion in this case was  $30^{\circ}\text{C}$ . The resulting paper had the following properties:

|                          |                         |
|--------------------------|-------------------------|
| carrier resistance       | 1.8 - 2.2 sec.          |
| smoothness (Bekk tester) | 100 - 110 sec.          |
| density                  | 0.82 g./cm <sup>3</sup> |

Transferring of images developed by liquid developer was effected on the resulting paper by using a commercially available liquid developing copier of transferring type (NP-L7, trade name, manufactured by Canon (K. K.). The result of transferring was good, but the fixation is a little bad.

When sample A is not subjected to a machine calender treatment (sample B), the properties were as shown below:

|                    |                         |
|--------------------|-------------------------|
| carrier resistance | 0.8 - 1.0 sec.          |
| smoothness         | 25 - 29 sec.            |
| density            | 0.78 g./cm <sup>3</sup> |

The sample B having the above mentioned properties were used for transferring under the same conditions as sample A, but satisfactory transferring was not effected.

In place of vinyl acetate emulsion used in sample A, there was used a vinyl acetate-butyl acrylate (90:10) copolymer emulsion to produce a transferring paper. The Tg value of the emulsion was 22°C. Properties of the resulting transferring paper were:

|                    |                           |
|--------------------|---------------------------|
| Carrier resistance | 3.8 - 4.2 sec.            |
| smoothness         | 110 - 120 sec.            |
| density            | 0.82 g./cm <sup>3</sup> . |

The transferring property and fixing property were excellent.

#### EXAMPLE 2

Transferring papers of various Tg values as shown below were prepared by using styrene series emulsion and compared with each other.

Table 3

| Copolymer component        | Ratio of components | Tg value |
|----------------------------|---------------------|----------|
| (1) Styrene-butyl acrylate | 100/0               | 90°C     |
| (2) do.                    | 75/25               | 48°C     |
| (3) do.                    | 60/40               | 25°C     |
| (4) do.                    | 50/50               | 8°C      |
| (5) do.                    | 0/100               | -57°C    |

25 30

The emulsions 1 - 4 in Table 5 above were mixed with an aqueous solution of polyvinylalcohol and clay at a ratio of 5:1:4 (as solid), impregnated in a base paper (60 g./m<sup>2</sup>) containing 20% of titanium oxide based on pulp at an amount of 8 g./m<sup>2</sup>, and subjected to super calender treatment (for example J, K, L and M). Sample M was further subjected to an intensified super calender treatment to increase the smoothness and thus samples N and O were produced. Properties of these samples are shown in Table 6.

Titanium oxide serves to prevent the formation of transparency to a great extent when the carrier penetrates the paper, and in case of samples N and O of good carrier resistance the pinhole is not noticeable. Therefore, the resulting transferring papers are also suitable for both side transferring.

Table 6

| Sample No. | Tg value of emulsion (°C) | Carrier resistance (sec.) | Smoothness (sec.) | Density (g./cm <sup>3</sup> ) | Transferring property | Fixing property |
|------------|---------------------------|---------------------------|-------------------|-------------------------------|-----------------------|-----------------|
| J          | 99°C                      | 17-20                     | 130-150           | 0.83                          | △                     | X               |
| K          | 30°C                      | 3.8-4.2                   | 150-170           | 0.85                          | ○                     | △               |
| L          | 25°C                      | 4.9-5.3                   | 150-180           | 0.85                          | ○                     | ○               |
| M          | -27°C                     | 8.9-9.5                   | 170-200           | 0.87                          | ○                     | ○               |
| N          | -27°C                     | 10.2-10.8                 | 230-250           | 0.92                          | ○                     | ○               |
| O          | -27°C                     | 11.5-12.2                 | 320-340           | 0.94                          | ○                     | △               |

The emulsions 1 - 5 in Table 3 were mixed with titanium oxide at a ratio of 2 to 1 (by weight, as solid), coated on a base paper (60 g./m<sup>2</sup>) at an amount of 3 g./m<sup>2</sup> by off-machine coating, subjected to a calender treatment to produce samples, E, F, G, H, and I, and carrier resistance, smoothness transferring property and fixing property of the resulting samples were measured. The results are shown in Table 4.

The density was 0.81 - 0.82 g./cm<sup>3</sup>. for each sample.

45 50

#### EXAMPLE 4

Vinyl acetate-butyl acrylate copolymer emulsion having the following Tg value was mixed with clay at a ratio of 2:1 (as solid), coated on a base paper (64 g./m<sup>2</sup>) at an amount of 8 - 10 g./m<sup>2</sup>. (as solid) and subjected to a calender treatment.

Properties of the resulting samples P, Q and R are shown in Table 7.

The density was 0.82 - 0.83 g./cm<sup>3</sup>. for each sample.

Table 7

| Sample No. | Composition of copolymer     | Composition ratio | Tg value (°C) | Carrier resistance (sec.) | Smooth (sec.) | Transferring property | Fixing property |
|------------|------------------------------|-------------------|---------------|---------------------------|---------------|-----------------------|-----------------|
| P          | Vinyl acetate-butyl acrylate | 75/25             | 8             | 4.3-4.7                   | 120-130       | ○                     | ○               |
| Q          | do.                          | 60/40             | -5            | 4.5-5.0                   | 130-140       | ○                     | ○               |
| R          | do.                          | 50/50             | -14           | 4.8-5.2                   | 135-145       | ○                     | ○               |

Table 4

| Sample No. | Tg value of emulsion | Carrier resistance (sec.) | Smoothness (sec.) | Transferring property | Fixing property |
|------------|----------------------|---------------------------|-------------------|-----------------------|-----------------|
| E          | 90°C                 | less than 1.5             | 60-65             | X                     | X               |
| F          | 48°C                 | 1.8-2.2                   | 70-75             | △                     | △               |
| G          | 25°C                 | 3.7-4.2                   | 90-100            | ○                     | ○               |
| H          | 8°C                  | 4.8-5.2                   | 110-120           | ○                     | ○               |
| I          | -57°C                | 5.1-5.7                   | blocking          | —                     | sticky          |

65

#### EXAMPLE 5

Vinyl acetate-butyl acrylate copolymer emulsion (sample Q, Tg value of -5°C) as used in Example 4 was mixed with clay at a ratio as shown in Table 8 below and coated on one side of a base paper (54 g./m<sup>2</sup>) at an amount of about 4 g./m<sup>2</sup>. On the other side of the base paper was preliminarily coated a mixture of vinyl acetate emulsion (Tg value of 35°C) and clay (1:7) at an amount of about 4 g./m<sup>2</sup>. The paper thus coated on both sides was subjected to calender.

Table 8

| Binder/clay ratio | Carrier resistance (sec.) | Smooth (sec.) | Density (g./cm <sup>3</sup> .) | Transferring property | Fixing property     |
|-------------------|---------------------------|---------------|--------------------------------|-----------------------|---------------------|
| 700/100           | 15.2-17.0                 | 180-200       | 0.85                           | ○                     | △ (very sticky)     |
| 500/100           | 12.5-14.0                 | 170-190       | 0.88                           | ○                     | ○ (somewhat sticky) |
| 400/100           | 11.3-12.5                 | 190-210       | 0.88                           | ○                     | ○                   |
| 100/100           | 6.5-7.8                   | 230-240       | 0.93                           | ○                     | ○                   |
| 50/100            | 3.7-4.5                   | 270-290       | 0.95                           | ○                     | ○                   |
| 25/100            | 2.5-3.5                   | 320-340       | 0.98                           | ○                     | △                   |

## EXAMPLE 6

A mixture of SB latex (styrene-butadiene latex) and calcium carbonate (3:1, as solid) was coated on a paper (70 g./m<sup>2</sup>.) at an amount of 6-8 g./m<sup>2</sup>. (as solid, on 15 one side) and subjected to calender treatment. Tg value of the latex was 20°C.

in Table 9 below, clay and barium sulfate were mixed at a ratio of 5:4:1, coated on a base paper (60 g./m<sup>2</sup>.) at an amount of 5 g./m<sup>2</sup>. and subjected to calender treatment. Properties of the resulting transferring paper are shown in Table 9 below.

The density was 0.87 g./cm<sup>3</sup>. in each case.

Table 9

| Copolymer component    | Component ratio | Tg value (°C) | Carrier resistance | Smoothness | Transferring property | Fixation        |
|------------------------|-----------------|---------------|--------------------|------------|-----------------------|-----------------|
| ethylene-vinyl acetate | 4/6             | -28           | 4.5-5.0            | 170-190    | ○                     | ○               |
| do.                    | 5/5             | -39           | 5.2-5.6            | 200-220    | ○                     | ○               |
| do.                    | 6/4             | -49           | 5.9-6.5            | blocking   | —                     | somewhat sticky |

Properties of the resulting sample are as shown below:

|                    |                           |
|--------------------|---------------------------|
| carrier resistance | 4.0 - 4.5 sec.            |
| smoothness         | 210 - 250 sec.            |
| density            | 0.83 g./cm <sup>3</sup> . |

The resulting transferring paper gave a transferred image of sufficient density and sharpness and good fixation.

## EXAMPLE 7

Nonionic series emulsion of vinyl acetate-butyl acrylate copolymer (Tg value of -5°C), a higher polymer quaternary ammonium salt, a water soluble polyvinylalcohol and clay were mixed at a ratio of 5:1:1:5 (as solid, by weight), attached to a base paper (54 g./m<sup>2</sup>.) at an amount of 7-8 g./m<sup>2</sup>. by impregnation and subjected to calender treatment.

The transferring paper thus produced had the following properties:

|                    |                           |
|--------------------|---------------------------|
| carrier resistance | 5.2 - 5.8 sec.            |
| smoothness         | 80 - 85 sec.              |
| density            | 0.85 g./cm <sup>3</sup> . |

The transferring paper gave a transferred image of sufficient density and sharpness, and the fixation was also excellent.

## EXAMPLE 8

Vinyl acetate-ethylene copolymer emulsion as shown

1. A transferring paper for an electrophotographic process comprising developing an electric latent image 30 with a liquid developer and transferring the image thus developed to the transferring paper which comprises a base paper and a coating layer produced by coating on the base paper a coating agent composed of 100-400 parts (as solid) of a polymer emulsion having a second order transition temperature of from -40°C to 25°C as a binder, and 100 parts of a white inorganic filler of a particle size of less than 3 microns and selected from the group consisting of clay, titanium oxide, calcium carbonate and barium sulfate in the amount of 2-10 g./m<sup>2</sup> (as a solid), carrier resistance of the resulting transferring surface being 1.5-15 sec., smoothness of the resulting transferring surface being 30-300 sec. and density being 0.75-100 g./cm<sup>3</sup>.

2. A transferring paper according to claim 1 in which 45 the carrier resistance is 2-10 sec.

3. A transferring paper according to claim 1 in which the smoothness is 40-200 sec.

4. A transferring paper according to claim 1 in which the second order transition temperature ranges from 50 -30°C to 0°C.

5. A transferring paper according to claim 1 in which the polymer emulsion is an emulsion selected from the group consisting of polyvinyl acetate, vinyl acetate-ethylene copolymer, vinyl acetate-acrylic acid ester copolymer, styrene-acrylic acid ester copolymer, methacrylic acid ester-acrylic acid ester copolymer, and styrene-butadiene latex.

\* \* \* \* \*

UNITED STATES PATENT OFFICE  
CERTIFICATE OF CORRECTION

Patent No. 3,889,033 Dated June 10, 1975

Inventor(s) HIROSHI TANAKA, ET AL

It is certified that error appears in the above-identified patent and that said Letters Patent are hereby corrected as shown below:

Column 2, line 39 "blurried" should read --blurred--

Column 4, line 9 "g./m" should read --such--

Column 4, line 60, "different" should read --difficult--

Column 6, line 57, "Canon (K." should read --Canon K."

On the Cover Page, Right Column, Line 4, "Urancken" should read --Vrancken--

Signed and Sealed this

nineteenth Day of August 1975

[SEAL]

Attest:

**RUTH C. MASON**  
*Attesting Officer*

**C. MARSHALL DANN**  
*Commissioner of Patents and Trademarks*